

# UNITED STATES PATENT OFFICE.

BERTRAND S. SUMMERS, OF PORT HURON, MICHIGAN, ASSIGNOR, BY MESNE ASSIGNMENTS,  
TO INTERNATIONAL FLAX TWINE COMPANY, A CORPORATION OF MINNESOTA.

## PROCESS OF PREPARING FLAX YARN.

No. 895,123.

Specification of Letters Patent.

Patented Aug. 4, 1908.

Application filed November 1, 1906. Serial No. 341,651.

*To all whom it may concern:*

Be it known that I, BERTRAND S. SUMMERS, a citizen of the United States, residing at Port Huron, in the county of St. Clair 5 and State of Michigan, have invented certain new and useful Improvements in Processes of Preparing Flax Yarn, of which the following is a specification.

My invention relates to the method or 10 process of preparing unretted flax yarn after the same is spun and the object thereof is to so treat or prepare the flax yarn as to impart thereto additional strength, and to improve the color and appearance thereof. When 15 unretted flax fiber is spun into the yarn, it is more or less rough in appearance and contains more or less woody particles derived from the woody portion of the plant, which particles are known as shive. The shive im- 20 parts to the yarn a more or less crude appearance and the natural roughness of the fiber enhances this irregularity to such a degree as to make the yarn appear rough and irregular. I have discovered that when this un- 25 retted flax yarn is dampened during the balling operation and the same is allowed to stand in a dampened condition in the ball for a certain length of time, the yarn greatly improves in color as well as strength and that 30 the rough fibers become nicely laid in the yarn, besides which the shive and the yarn itself get practically the same color, so that the shive is not nearly as apparent in the 35 yarn. Moreover, this action has considerable of a bleaching tendency, resulting in a much more commercial yarn.

In order to aid the action above described, resulting from dampening, and to further enhance the strength of the yarn, I add to the 40 water certain ingredients which I find to be of material benefit. The ingredients which I preferably employ are glue and soft soap which are made into an aqueous solution by mixing with water, as hereinafter explained, 45 both the glue and soap being used, although some measure of my invention may be obtained if either one thereof were to be used alone. The glue adds materially to the strength of the fiber and greatly aids in laying the fuzz or rough fibers of the yarn, while the soap has a marked solvent action on the 50 coloring matter of the flax which greatly aids

in imparting a uniform appearance to the yarn as regards color, the soap also preventing the glue from sticking or cementing the 55 yarn together and thereby permitting the yarn to be readily unwound from the ball. While the proportions of these ingredients may be considerably varied, I prefer to use a mixture comprising substantially two parts 60 of glue, six parts of soap, and three parts of water, which ingredients are heated together until all are in solution, which is kept sufficiently warm to maintain the ingredients in a fluid condition.

Any convenient means whatsoever may be used in introducing the solution into the 65 yarn, and the same may be introduced at any desired stage after the spinning operation, the only precaution necessary being to 70 prevent the yarn from becoming too wet, it being found in practice that about ten per cent. of the weight of the yarn is a very suitable amount of the solution to be introduced 75 into the yarn. However, I prefer to introduce this solution into the yarn while it is passing from the bobbin onto the balling spindle, and this can be done either by means of a small roller working in a trough, or the 80 yarn can simply be passed over a sponge or piece of soft cloth such as felt, which has been moistened with the solution.

What I claim and desire to secure by Letters Patent is:

1. The process of preparing yarn which 85 consists in moistening unretted flax yarn and balling the same while in a moist condition.

2. The process of preparing yarn which 90 consists in moistening unretted flax yarn with an aqueous solution of glue and balling the same while in a moist condition.

3. The process of preparing yarn which 95 consists in moistening unretted flax yarn with an aqueous solution of soap and balling the same while in a moist condition.

4. The process of preparing yarn, which 99 consists in treating unretted flax yarn with an aqueous solution of glue and soap and balling the same while in a moist condition.

BERTRAND S. SUMMERS.

Witnesses:

THOMAS J. WHITE,  
E. S. Post.